# EUROPEAN PATENT SPECIFICATION

(11) **EP 0 057 759 B1**
(45) Date of publication and mention of the grant of the patent: **05.03.1986**
(21) Application number: 81108991.1
(22) Date of filing: 27.10.1981
(51) Int. Cl.: B41M 5/26, B41J 31/08

(54) **Thermal transfer printing resistive ribbon**
Widerstandsband für den Thermotransferdruck
Ruban à conductivité anisotropique pour l'impression par transfert thermique

(30) Priority: 06.02.1981 US 232070
(43) Date of publication of application: 18.08.1982
(73) Proprietor: International Business Machines Corporation, Armonk, N.Y. 10504 (US)
(72) Inventor: Niweigha, Tiefa Kingsley, San Jose California 95111 (US); Shattuck, Meredith David, Hollister California 95023 (US)
(74) Representative: Ahlman, Bertel

## Description

The present invention relates to resistive ribbons for use in thermal transfer printing onto a receptor surface.

Resistive ribbon thermal transfer printing is known in the art and is, very briefly, summarised in US―4,103,066, DE-2,842,772, FR-2,434,709 and GB-1,583,922, which disclose a resistive ribbon comprising a resistive polycarbonate layer or substrate with a transfer layer of wax, carbon black and a dye on one surface thereof.

The use in a resistive ribbon for thermal transfer printing of a "hold-off" layer as the layer closest to the receptor surface to be printed upon, is disclosed in European patent application No. 81103625.0, publication No. EP-0042954, filed before but published after the priority date of this application.

According to EP0042954, the ordinary ink layer is overcoated with a second layer called a hold-off layer because it prevents or holds the ink from penetrating into the paper fibers. At the same time, the hold-off layer adheres to the paper sufficiently well so that the paper may be handled, creased and otherwise subjected to ordinary wear without smearing or deterioration of the print quality.

During the printing operation, the hold-off layer comes into contact with the substrate being printed upon, for example, paper. The ink layer is simultaneously transferred with the hold-off layer. The hold-off.layer is thus deposited on the paper beneath the ink layer. Thus, the hold-off layer serves to make subsequent correction of the printing easier by preventing the ink from penetrating into the pores of the substrate paper being printed upon.

The use of a polyvinyl acetate layer in a pressure sensitive ribbon is disclosed in US3481761.

The present invention is defined in the attached claims.

The layer of polyvinyl acetate may serve as the transfer layer. In such case, the layer of polyvinyl acetate contains a pigment, such as carbon, and/ or one or more colouring dyes, and selected portions are transferred from the resistive ribbon to the receptor surface during printing to serve as the ink.

The layer of polyvinyl acetate layer may be used as a hold-off layer. In such case, the layer is uncoloured and serves to make subsequent correction of printing easier. When the polyvinyl acetate layer is used as a hoid-off tayer, it is used in conjunction with a transfer layer, which acts as the ink, and contains pigment and/or colouring material. The hold-off layer serves to prevent the ink from penetrating the pores of the receptor surface being printed upon. The polyvinyl acetate hold-off layer may be used with any of the known useful transfer layers, for example, a layer of polymerized fatty acid polyamide, as disclosed in GB-2,010,515.

Most preferred, however, is the use of a polyvinyl acetate uncoloured hold-off layer with a pigmented transfer layer of polyvinyl acetate.

The use of a polyvinyl acetate layer in a resistive ribbon according to the present invention, gives the advantages of rub resistance, waterfastness and correctability, while at the same time providing excellent print quality. An additonal advantage is that such a layer is capable of formulation by water based application, rather than from an organic solvent. Thus, the use of organic solvents is avoided and an ecological advantage achieved.

The polyvinyl acetate layer, whether serving as hold-off layer or transfer layer, is suitable for use. with any of the resistive layers and conductive layers known in the thermal transfer resistive ribbon making art. The polycarbonate ribbon of US-4,103,066 is one preferred resistive layer.

In general, the polyvinyl acetate layer, when used as a hold-off layer, should be from about 0.1 to 10 microns in thickness, and preferably from about 1 to about 2 microns. When the polyvinyl acetate layer is used as a transfer layer, it should be from about 1 to about 5 microns thick.

Polyvinyl acetate suitable for use in the present invention is available commercially from a number of sources. For example, polyvinyl acetate latex is available from Union Carbide Corporation under the trademark Ucar Vehicle 4029. Carbon pigments suitable for use in conjunction with polyvinyl acetate for the transfer layer of the present invention are also readily available commercially. For example, Aqua Blak, a brand of carbon from the Borden company.

The following additional examples illustrate the invention, but many variations are possible without departing from the scope of the claims.

### Example 1

A transfer layer was prepared by applying:
30 parts polyvinyl acetate latex;
40 parts water; and
7.5 parts carbon,

to a metallized polyurethane/polyester crosslinked resistive layer. The layer was dried with heat, and the ribbon was evaluated on a resistive ribbon thermal transfer robot. Excellent quality print was obtained at 35 to 40 milliamps current.

### Example 2

A transfer layer was prepared as in Example 1, except that the formulation was applied to a metallized resistive layer of polycarbonate.

The ribbon was evaluated on a resistive ribbon thermal transfer robot and was found to produce excellent quality print at 30 to 35 milliamps current.

### Example 3

A hold-off layer was prepared by applying polyvinyl acetate latex in water to a polyamide transfer layer on a polycarbonate layer or substrate of a resistive ribbon. A thin clear layer of uncoloured polyvinyl acetate was formed on the polyamide ink surface of the ribbon.

The ribbon was printed onto paper. The latex layer prevented penetration of the ink into the paper. The print thus formed was lifted off the paper with adhesive tape, demonstrating the correctability of the material.

## Claims

1. A resistive ribbon for thermal transfer printing comprising a resistive substrate layer and an ink layer covered by another layer, characterized in that said ribbon is a correctable thermal transfer ribbon, that said another layer is transferable with the ink layer to the receptor surface being printed upon, that the another layer prevents penetration of the ink into the receptor surface and that the another layer is a polyvinyl acetate layer.

2. A ribbon according to claim 1, in which the ink layer is a layer of coloured polyvinyl acetate.

3. A ribbon according to claim 1, in which said another layer is from 0.1 to 10 microns thick.

4. A ribbon according to claim 3, in which said another layer is from 1 to 2 microns thick.

5. A ribbon according to claim 2, in which the coloured polyvinyl acetate ink layer is from 1 to 5 microns thick.

6. A ribbon according to claim 5 in which the polyvinyl acetate ink layer also includes polyethylene oxide.

## Revendications

1. Un ruban résistif pour impression par transfert thermique comprenant une couche ou substrat résistif et une couche d'encre recouverte par une autre couche, caractérisé en ce que ledit ruban est un ruban de transfert thermique pouvant être corrigé, en ce que ladite autre couche est transférable avec la couche d'encre sur la surface réceptrice en train d'être imprimée, en ce que l'autre couche empêche une pénétration de l'encre dans la surface réceptrice et en ce que l'autre couche est une couche d'acétate de polyvinyle.

2. Un ruban conforme à la revendication 1, dans lequel la couche d'encre est une couche d'acétate de polyvinyle coloré.

3. Un ruban conforme à la revendication 1, dans lequel ladite autre couche a une épaisseur comprise entre 0,1 et 10 microns.

4. Un ruban conforme à la revendication 3, dans lequel ladite autre couche a une épaisseur comprise entre 1 et 2 microns.

5. Un ruban conforme à la revendication 2, dans lequel la couche d'encre en acétate de polyvinyle coloré a une épaisseur comprise entre 1 et 5 microns.

6. Un ruban conforme à la revendication 5, dans lequel la couche d'encre en acétate de polyvinyle contient également de l'oxyde de polyéthylène.

## Patentansprüche

1. Widerstandsband für einen Thermotransferdruck, mit einer Widerstands-Substratschicht und einer von einer weiteren Schicht abgedeckten Tintenschicht, dadurch gekennzeichnet, daß das Band ein korigierbares Thermotransferband ist, daß die weitere Schicht zusammen mit der Tintenschicht auf die Rezeptorfläche, auf welcher gedruckt wird, übertragbar ist, das die weitere Schicht ein Eindringen der Tinte in die Rezeptorfläche verhindert und daß die weitere Schicht eine Polyvinylacetat-Schicht ist.

2. Band nach Anspruch 1, bei welchem die Tintenschicht eine Schicht aus gefärbtem Polyvinylacetat ist.

3. Band nach Anspruch 1, bei welchem die weitere Schicht zwischen 0,1 und 10 unn dick ist.

4. Band nach Anspruch 3, bei welchem die weitere Schicht zwischen 1 und 2 um dick ist.

5. Band nach Anspruch 2, bei welchem die Tintenschicht aus gefärbtem Polyvinylacetat zwischen 1 und 5 um dick ist.

6. Band nach Anspruch 5, bei welchem die Polyvinylacetat-Tintenschicht auch Polyethylenoxid enthält.
